# EUROPEAN PATENT SPECIFICATION

(11) **EP 1 228 167 B1**
(45) Date of publication and mention of the grant of the patent: **30.06.2010**
(21) Application number: 00965111.8
(22) Date of filing: 18.09.2000
(51) Int. Cl.: C10G 11/05

(54) **USE OF SULFUR REDUCTION AGENT IN FLUID CATYLYTIC CRACKING**
VERWENDUNG EINES MITTELS ZUR REDUKTION DES SCHWEFELGEHALTES IN EINEM KATALYTISCHEN FLUIDCRACKING PROZESS
UTILISE D' UN AGENT DE REDUCTION DU SOUFRE CONTENU DANS L'ESSENCE LORS DU CRAQUAGE CATALYTIQUE FLUIDE

(30) Priority: 20.09.1999 US 399637; 28.08.2000 US 649627
(43) Date of publication of application: 07.08.2002
(62) Divisional of application: 10003379.4
(73) Proprietor: W.R. GRACE & CO.-CONN., New York, NY 10036 (US); Mobil Oil Corporation, Fairfax, VA 22037 (US)
(72) Inventor: ROBERIE, Terry, G., Ellicott City, MD 21042 (US); KUMAR, Ranjit, Clarksville, MD 21029 (US); ZIEBARTH, Michael, S., Columbia, MD 21044 (US); CHENG, Wu-Cheng, Ellicott City, MD 21042 (US); ZHAO, Xinjin, Woodbine, MD 21797 (US); BHORE, Nazeer, Gaithersburg, MD 20878 (US)
(74) Representative: UEXKÜLL & STOLBERG
(86) International application number: PCT/US2000/025533
(87) International publication number: WO 2001/021732

(56) References cited:
- GB-A- 2 341 191
- US-A- 4 642 177
- US-A- 5 399 327
- US-A- 5 618 406

## Description

### FIELD OF THE INVENTION

This invention relates to the reduction of sulfur in gasoline and other petroleum products produced by a catalytic cracking process. The invention provides a catalytic composition for reducing product sulfur and a process for reducing product sulfur using this composition.

### CROSS-REFERENCE TO RELATED US APPLICATIONS

This application is a continuation in part to US Application Serial No. 09/399,637, filed September 20, 1999.

This application is related to US Application Serial No. 09/144,607, filed August 31, 1998.

This application is also related to US application Serial Nos. 09/221,539 and 09/221,540, both filed December 28, 1998.

### BACKGROUND OF THE INVENTION

Catalytic cracking is a petroleum refining process which is applied commercially on a very large scale. A majority of the refinery gasoline blending pool in the United States is produced by this process, with almost all being produced using the fluid catalytic cracking (FCC) process. In the catalytic cracking process heavy hydrocarbon fractions are converted into lighter products by reactions taking place at elevated temperature in the presence of a catalyst, with the majority of the conversion or cracking occurring in the vapor phase. The feedstock is thereby converted into gasoline, distillate and other liquid cracking products as well as lighter gaseous cracking products of four or less carbon atoms per molecule. The gas partly consists of olefins and partly of saturated hydrocarbons.

During the cracking reactions some heavy material, known as coke, is deposited onto the catalyst. This reduces the activity of the catalyst and regeneration is desired. After removal of occluded hydrocarbons from the spent cracking catalyst, three characteristic steps of the catalytic cracking can be therefore be distinguished: a cracking step in which the hydrocarbons are converted into lighter products, a stripping step to remove hydrocarbons adsorbed on the catalyst and a regeneration step to burn off coke from the catalyst. The regenerated catalyst is then reused in the cracking step.

Catalytic cracking feedstocks normally contain sulfur in the form of organic sulfur compounds such as mercaptans, sulfides and thiophenes. The products of the cracking process correspondingly tend to contain sulfur impurities even though about half of the sulfur is converted to hydrogen sulfide during the cracking process, mainly by catalytic decomposition of non-thiophenic sulfur compounds. The distribution of sulfur in the cracking products is dependent on a number of factors including feed, catalyst type, additives present, conversion and other operating conditions but, in any event a certain proportion of the sulfur tends to enter the light or heavy gasoline fractions and passes over into the product pool. With increasing environmental regulation being applied to petroleum products, for example in the Reformulated Gasoline (RFG) regulations, the sulfur content of the products has generally been decreased in response to concerns about the emissions of sulfur oxides and other sulfur compounds into the air following combustion processes.

One approach has been to remove the sulfur from the FCC feed by hydrotreating before cracking is initiated. While highly effective, this approach tends to be expensive in terms of the capital cost of the equipment as well as operationally since hydrogen consumption is high. Another approach has been to remove the sulfur from the cracked products by hydrotreating. Again, while effective, this solution has the drawback that valuable product octane may be lost when the high octane olefins are saturated.

From the economic point of view, it would be desirable to achieve sulfur removal in the cracking process itself since this would effectively desulfurize the major component of the gasoline blending pool without additional treatment. Various catalytic materials have been developed for the removal of sulfur during the FCC process cycle, but, so far most developments have centered on the removal of sulfur from the regenerator stack gases. An early approach developed by Chevron used alumina compounds as additives to the inventory of cracking catalyst to adsorb sulfur oxides in the FCC regenerator; the adsorbed sulfur compounds which entered the process in the feed were released as hydrogen sulfide during the cracking portion of the cycle and passed to the product recovery section of the unit where they were removed. See Krishna et al, Additives Improve FCC Process, Hydrocarbon Processing, November 1991, pages 59-66 and US-A-4 642 177. The sulfur is removed from the stack gases from the regenerator but product sulfur levels are not greatly affected, if at all.

An alternative technology for the removal of sulfur oxides from regenerator stack gases is based on the use of magnesium-aluminum spinels as additives to the circulating catalyst inventory in the FCCU. Under the designation DESOX™ used for the additives in this process, the technology has achieved a notable commercial success. Exemplary patents disclosing this type of sulfur removal additives include U.S. Patent Nos. 4,963,520; 4,957,892; 4,957,718; 4,790,982 and others. Again, however, product sulfur levels are not greatly reduced.

A catalyst additive for the reduction of sulfur levels in the liquid cracking products was proposed by Wormsbecher and Kim in U.S. Patents 5,376,608 and 5,525,210, using a cracking catalyst additive of an alumina-supported Lewis acid for the production of reduced-sulfur gasoline but this system has not achieved significant commercial success.

In US Application Serial No. 09/144,607, filed August 31, 1998, catalytic materials are described for use in the catalytic cracking process which are capable of reducing the content of the liquid products of the cracking process. These sulfur reduction catalysts comprise, in addition to a porous molecular sieve component, a metal in an oxidation state above zero within the interior of the pore structure of the sieve. The molecular sieve is in most cases a zeolite and it may be a zeolite having characteristics consistent with the large pore zeolites such as zeolite beta or zeolite USY or with the intermediate pore size zeolites such as ZSM-5. Non-zeolitic molecular sieves such as MeAPO-5, MeAPSO-5, as well as the mesoporous crystalline materials such as MCM-41 may be used as the sieve component of the catalyst. Metals such as vanadium, zinc, iron, cobalt, and gallium were found to be effective for the reduction of sulfur in the gasoline, with vanadium being the preferred metal. The amount of the metal component in the sulfur reduction additive catalyst is normally from 0.2 to 5 weight percent, but amounts up to 10 weight percent were stated to give some sulfur removal effect. The sulfur reduction component may be a separate particle additive or part of an integrated cracking/sulfur reduction catalyst. When used as a separate particle additive catalyst, these materials are used in combination with an active catalytic cracking catalyst (normally a faujasite such as zeolite Y and REY, especially as zeolite USY and REUSY) to process hydrocarbon feedstocks in the FCC unit to produce low-sulfur products.

In US Application Serial Nos. 09/221,539 and 09/221,540, both filed December 28, 1998, sulfur reduction catalysts similar to the one described in Application No. 09/144,607 were described, however, the catalyst compositions in those applications also comprise at least one rare earth metal component (e.g. lanthanum) and a cerium component, respectively. The amount of the metal component in the sulfur reduction catalysts is normally from 0.2 to 5 weight percent, but amounts up to 10 weight percent were suggested to give some sulfur removal effect.

In US Application Serial No. 09/399,637, filed September 20, 1999, an improved catalytic cracking process for reducing the sulfur content of the liquid cracking products, especially cracked gasoline, produced from hydrocarbon feed containing organosulfur compounds is described. The process employs a catalyst system having a sulfur reduction component containing porous catalyst and a metal component in an oxidation state greater than zero. The sulfur reduction activity of the catalyst system is increased by increasing average oxidation state of the metal component by an oxidation step following conventional catalyst regeneration. The catalyst is normally a molecular sieve such as zeolite Y, REY, USY, RESUY, Beta or ZSM-5. Non-zeolitic molecular sieves such as MeAPO-5, MeAPSO-5, as well as the mesoporous crystalline materials such as MCM-41 and MCM-48 may also be used as the sieve component of the catalyst. Amorphous and paracrystalline materials such as amorphous refractory inorganic oxides of Group 2, 4, 13 and 14 of the periodic table, for example, Al₂O₃, SiO₂, ZrO₂, TiO₂, MgO and mixtures thereof, and paracrystalline materials such as transitional aluminas, are also contemplated as useful support components for the metal component of the sulfur reduction catalysts. The metal component is normally a metal of Groups 5, 7, 8, 9, 12 or 13 of the Periodic Table, preferably vanadium or zinc. The amount of metal in the sulfur reduction component is normally from 0.1 to 10 weight percent (as metal, relative to the weight of the support component), however, amounts up to 10 weight percent were stated to have some sulfur removal effect. The sulfur reduction component may be a separate particle additive or part of an integrated cracking/sulfur reduction catalyst. A system for increasing the oxidation state of the metal component of a gasoline sulfur reduction additive is also described.

There continues to exist a need for effective ways to further reduce the sulfur content of gasoline and other liquid cracking products. The present invention was developed in response to this need.

### SUMMARY OF THE INVENTION

The present invention is directed to the use of a sulfur reduction additive in a fluid catalytic cracking process as defined in claim 1. The used additive is capable of improving the reduction in the sulfur content of liquid products produced by the cracking process, in particular, the gasoline and middle distillate cracking fractions. The present sulfur reduction additives are similar to additives described in US Application Nos. 09/144,607, 09/221,539 and 09/221,540, in that the additive materials employ a sulfur reduction component containing a metal component in an oxidation state greater than zero, i.e. vanadium. The sulfur reduction component in US Application Nos. 09/144,607, 09/221,539 and 09/221,540 comprises a molecular sieve (preferably, a zeolitic molecular sieve) which contains a metal component in an oxidation state above zero, i.e. vanadium, within the interior of the pore structure. In contrast, the sulfur reduction additives of the present invention, comprise a non-molecular sieve support material which contains a relatively high content of vanadium metal. It has been found that the use of a non-molecular sieve catalyst support in combination with a relatively high concentration of vanadium enhances the rate of transport of vanadium over the entire FCC catalyst inventory, thereby increasing the activity of the catalyst to remove sulfur.

According to the present invention, the sulfur reduction additives comprise a non-molecular sieve catalyst support material containing a high content of vanadium in an oxidation state greater than zero. The support material may be organic or inorganic in nature and may be porous or non-porous. Preferably, the support material is an amorphous or paracrystalline inorganic oxide such as, for example, Al₂O₃, SiO₂, clays or mixtures thereof. The sulfur reduction additives are used as a separate particle additive in combination with the conventional catalytic cracking catalyst (normally a faujasite such as zeolite Y) to process hydrocarbon feedstocks in the fluid catalytic cracking (FCC) unit to produce low-sulfur gasoline and other liquid cracking products, such as, for example, light cycle oil that can be used as a low sulfur diesel blend component or as heating oil.

Accordingly, it is an advantage of the present invention to provide improved liquid product sulfur reduction when compared to the sulfur reduction activity of a base FCC catalyst conventionally used in the catalyst cracking process.

It is also an advantage of the present invention to provide for the rapid dispersion of vanadium over the entire cracking catalyst inventory used in a catalytic cracking process, thereby enhancing the removal of sulfur components from cracked hydrocarbon products.

An additional advantage of the present invention is to provide sulfur reduction additive compositions having improved product sulfur reduction at lower additive levels than heretoafore used for conventional sulfur reduction additives, including vanadium/zeolite sulfur reduction additives disclosed in related US Application Nos. 09/144,607, 09/221,539 and 09/221,540.

### DETAIL DESCRIPTION OF THE INVENTION

For purposes of this invention the term "high vanadium content" or "high content of vanadium" is used herein to indicate a vanadium content of greater than 1.5 weight percent (as metal, relative to the total weight of the additve material).

The term "molecular sieve" is used herein to designate a class of polycrystalline materials that exhibits selective sorption properties which separates components of a mixture on the basis of molecular size and shape differences, and have pores of uniform size, i.e., from about 3Å to approximately 100 Å, which pore sizes are uniquely determined by the unit structure of the crystals. Materials such as activated carbons, activated alumina and silica gels are specifically excluded since they do not possess an ordered crystalline structure and consequently have pores of a non-uniform size. The distribution of the pore diameters of such material may be narrow (generally from about 20Å to about 50Å) or wide (ranging from about 20Å to several thousand Å) as in the case for some activated carbons. See R. Szostak, Molecular Sieves: Principles of Synthesis and Identification, pp. 1-4 and D.W. Breck, Zeolite Molecular Sieves, pp.1-30. A molecular sieve framework is based on an extensive three-dimensional network of oxygen atoms containing generally tetrahedral type-sites. In addition to the Si⁺⁴ and Al⁺³ that compositionally define a zeolite molecular sieves, other cations also can occupy these sites. These need not be iso-electronic with Si⁺⁴ or Al⁺³, but must have the ability to occupy framework sites. Cations presently known to occupy these sites within molecular sieve structures include but are not limited to Be, Mg, Zn, Co, Fe, Mn, Al, B, Ga, Fe, Cr, Si. Ge, Mn, Ti, and P. Another class of materials intended to fall within the scope of molecular sieve includes mesoporous crystalline materials exemplified by the MCM-41 and MCM-48 materials. These mesoporous crystalline materials are described in U.S. Patent Nos. 5,098,684; 5,102,643; and 5,198,203.

In accordance with the present invention, the sulfur content of the gasoline portion of the liquid cracking products, is effectively brought to lower and more acceptable levels by carrying out the catalytic cracking in the presence of the sulfur reduction additives comprising a high content of vanadium incorporated into a non-molecular sieve catalyst support material. While the mechanism by which the high vanadium-containing additives act to enhance removal of sulfur components normally present in cracked hydrocarbon products is not precisely understood, it is believed that the additive acts to rapidly transport vanadium over the entire cracking catalyst inventory. Such an increased dispersion of vanadium permits a more efficient rate of removal of liquid product sulfur than obtainable when using a base or conventional cracking catalyst alone or in combination with conventional sulfur reduction additives heretoafore used in catalyst cracking processes.

### FCC Process

The present sulfur removal additives are used as a component of the circulating inventory of catalyst in the catalytic cracking process, which these days is almost invariably the FCC process. For convenience, the invention will be described with reference to the FCC process although the present additives could be used in the older moving bed type (TCC) cracking process with appropriate adjustments in particle size to suit the requirements of the process. Apart from the addition of the present additive to the catalyst inventory and some possible changes in the product recovery section, discussed below, the manner of operating the process will remain unchanged. Thus, conventional FCC catalysts may be used, for example, zeolite based catalysts with a faujasite cracking component as described in the seminal review by Venuto and Habib, Fluid Catalytic Cracking with Zeolite Catalysts, Marcel Dekker, New York 1979, ISBN 0-8247-6870-1 as well as in numerous other sources such as Sadeghbeigi, Fluid Catalytic Cracking Handbook, Gulf Publ. Co. Houston, 1995, ISBN 0-88415-290-1.

Somewhat briefly, the fluid catalytic cracking process in which the heavy hydrocarbon feed containing the organosulfur compounds will be cracked to lighter products takes place by contact of the feed in a cyclic catalyst recirculation cracking process with a circulating fluidizable catalytic cracking catalyst inventory consisting of particles having a size ranging from about 20 to about 100 microns. The significant steps in the cyclic process are:
(i) the feed is catalytically cracked in a catalytic cracking zone, normally a riser cracking zone, operating at catalytic cracking conditions by contacting feed with a source of hot, regenerated cracking catalyst to produce an effluent comprising cracked products and spent catalyst containing coke and strippable hydrocarbons;
(ii) the effluent is discharged and separated, normally in one or more cyclones, into a vapor phase rich in cracked product and a solids rich phase comprising the spent catalyst;
(iii) the vapor phase is removed as product and fractionated in the FCC main column and its associated side columns to form liquid cracking products including gasoline;
(iv) the spent catalyst is stripped, usually with steam, to remove occluded hydrocarbons from the catalyst, after which the stripped catalyst is oxidatively regenerated to produce hot, regenerated catalyst which is then recycled to the cracking zone for cracking further quantities of feed.

The present sulfur reduction additives are used in the form of a separate particle additive which is added to the main cracking catalyst in the FCCU. The cracking catalyst will normally be based on a faujasite zeolite active cracking component, which is conventionally zeolite Y in one of its forms such as calcined rare-earth exchanged type Y zeolite (CREY), the preparation of which is disclosed in U.S. Patent No. 3,402,996, ultrastable type Y zeolite (USY) as disclosed in U.S. Patent No. 3,293,192, as well as various partially exchanged type Y zeolites as disclosed in U.S. Patents Nos. 3,607,043 and 3,676,368. The active cracking component is routinely combined with a matrix material such as alumina in order to provide the desired mechanical characteristics (attrition resistance etc.) as well as activity control for the very active zeolite component or components. The particle size of the cracking catalyst is typically in the range of 10 to 120 microns for effective fluidization. As a separate particle additive, the sulfur reduction additive is normally selected to have a particle size comparable with that of the cracking catalyst so as to prevent component separation during the cracking cycle. In general the particle size of the sulfur reduction additive is in the range of about 10 to about 200 microns, preferably, about 20 to about 120 microns.

### Sulfur Reduction Component

According to the present invention, the sulfur reduction additives comprise non-molecular sieve support materials as defined in the claims having a high content of vanadium. In one embodiment of the invention, the support materials are amorphous and paracrystalline support materials, namely refractory inorganic oxides of Groups 4, 13 and 14 of the Periodic Table. Suitable refractory inorganic oxides include, but are not limited to, Al₂O₃, SiO₂, TiO₂, clay (e.g. kaolin, bentonite, hectorite, montmorillonite and the like) and mixtures thereof. Preferably, the support materials are selected from the group consisting of Al₂O₃, SiO₂, clay (preferably kaolin) and mixtures thereof. Most preferably, the support material is alumina.

In another embodiment of the invention, the support material is an activated carbon. Support materials in accordance with the invention may be used alone or in combination to prepare sulfur reduction additives in accordance with the invention.

The amount of vanadium metal contained in sulfur reduction additives in accordance with the invention catalyst is normally from about 2.0 to about 20 weight percent, typically from about 3 to about 10 weight percent, most preferably from about 5 to about 7 weight percent (metal, based on the total weight of the additive). Vanadium may be added to the support in any suitable manner sufficient to adsorb and/or absorb a suitable vanadium containing compound onto or into the support material.

In one embodiment, the sulfur reduction additives are prepared by treating the support material with an aqueous or non-aqueous solution of a suitable vanadium compound to impregnate the vanadium compound into or onto the surface of the support material. Alternatively, vanadium may be added to the support by spray drying an aqueous slurry containing the support material and the desired vanadium compound. Non-limiting example of suitable vanadium compounds useful to prepare additives in accordance with the invention include, but are not limited to, vanadium oxalate, vanadium sulfate, organometallic vanadium complexes (e.g. vanadyl naphthenate), vanadium halides and oxyhalides (e.g. vanadium chlorides and oxychorides) and mixtures thereof.

Following addition of the vanadium component, the support material is dried and calcined, typically at temperatures ranging from about 100 to about 800 °C.

### Sulfur Reduction Catalyst Use

The sulfur reduction additives of the invention are used as separate particle additives to permit optimization of the transport of vanadium to the cracking catalyst inventory. Generally, the additives of the invention are used in an amount sufficient to increase the amount of vanadium on the cracking catalyst by about 100 to about 10,000 ppm, preferably about 500 to about 5000 ppm, most preferably about 1000 to about 2000 ppm, relative to the amount of vanadium initially present on the cracking catalyst. As will be understood by one skilled in the art, the amount of vanadium transported from the additive to the catalyst is readily determined by separating the additive from the cracking catalyst by skeletal density differences and analyzing each fraction for vanadium content after subjection to catalytic cracking condition in the presence of the additive.

The sulfur reduction additive is typically used in an amount from about 0.1 to about 10 weight percent of the cracking catalyst inventory in the FCCU; preferably, the amount will be from about 0.5 to about 5 weight percent. About 2 weight percent represents a norm for most practical purposes. The additive may be added in the conventional manner, with make-up catalyst to the regenerator or by any other convenient method. The additive remains active for sulfur removal for extended periods of time although very high sulfur feeds may result in loss of sulfur removal activity in shorter times.

Other catalytically active components may be present in the circulating inventory of catalytic material in addition to the cracking catalyst and the sulfur removal additive. Examples of such other materials include the octane enhancing catalysts based on zeolite ZSM-5, CO combustion promoters based on a supported noble metal such as platinum, stack gas desulfurization additives such as DESOX™ (magnesium aluminum spinel), vanadium traps and bottom cracking additives, such as those described in Krishna, Sadeghbeigi, *op cit* and Scherzer, Octane Enhancing Zeolitic FCC Catalysts, Marcel Dekker, New York, 1990, ISBN 0-8247-8399-9. These other components may be used in their conventional amounts.

The effect of the present additives is to reduce the sulfur content of liquid cracking products, especially the light and heavy gasoline fractions, although reductions are also noted in the light cycle oil, making them more suitable for use as a diesel or home heating oil blend component. The sulfur removed by the use of the FCC catalyst is converted to the inorganic form and released as hydrogen sulfide which can be recovered in the normal way in the product recovery section of the FCCU in the same way as the hydrogen sulfide conventionally released in the cracking process. The increased load of hydrogen sulfide may impose additional sour gas/water treatment requirements but with the significant reductions in gasoline sulfur achieved, these are not likely to be considered limitative.

Very significant reductions in gasoline sulfur can be achieved by the use of the present catalysts, in some cases up to about 80 % relative to the base case using a conventional cracking catalyst, at constant conversion, using the preferred form of the catalyst described above. Gasoline sulfur reduction of 10 to 60 % is readily achievable with additives according to the invention, as shown by the Examples below. The extent of sulfur reduction may depend on the original organic sulfur content of the cracking feed, with the greatest reductions achieved with the higher sulfur feeds. Sulfur reduction may be effective not only to improve product quality but also to increase product yield in cases where the refinery cracked gasoline end point has been limited by the sulfur content of the heavy gasoline fraction; by providing an effective and economical way to reduce the sulfur content of the heavy gasoline fraction, the gasoline end point may be extended without the need to resort to expensive hydrotreating, with a consequent favorable effect on refinery economics. Removal of the various thiophene derivatives which are refractory to removal by hydrotreating under less severe conditions is also desirable if subsequent hydrotreatment is contemplated.

In order to further illustrate the present invention and the advantages thereof, the following specific examples are given. The examples are given as specific illustrations of the claimed invention. It should be understood, however, that the invention is not limited to the specific details set forth in the examples. All part and percentages in the examples as well as the remainder of the specification are by weight unless otherwise specified.

The scope of the invention is not in any way intended to be limited by the examples set forth below. The examples include the preparation and use of sulfur reduction additives in accordance with the invention and evaluations of the performance of the additives to reduce sulfur in a catalytic cracking environment.

### EXAMPLES

### Example 1

### (Preparation of 2% Vanadium and 5% Vanadium on an Al₂O₃ Support)

A spray dried Al₂O₃ particle was prepared by peptizing a pseudoboehmite Al₂O₃ slurry with HCl, milling it with a Drais mill and then spray drying the milled slurry. The resulting spray dried alumina was calcined for 1 hour at 800° C.

The spray dried, calcined Al₂O₃ was then impregnated to incipient wetness with an aqueous vanadium oxalate solution. The concentration of vanadium oxalate in the solution was adjusted to produce a concentration of 2 wt% V and 5 wt% V on alumina.

The impregnated alumina was dried at 100° C and then calcined for 2 hours at 540° C.

### Example 2

### (Preparation of 6% V on an Al₂O₃ Support)

A spray dried, calcined Al₂O₃, prepared as described in Example 1 above, was impregnated to incipient wetness with an aqueous vanadium sulfate solution. The concentration of vanadium sulfate in solution was adjusted to produce 6 wt% V on alumina.

The impregnated material was dried at 120° C. The final material was analyzed by ICP and found to contain 5.4 wt% V, 0.1 wt% Na₂O, 11% SO₄. The surface area, as determined by N₂-BET, was 39 m²/g.

### Example 3

### (Preparation of 2.0 % V on a SiO₂-Clay Support)

A silica hydrogel (280-350 m²/g, 30-35% solids and 8.0-8.5 pH) was slurried in distilled water and sand milled to give a slurry which contained 14.8 wt% solids. A mixture of 13,514 g of the milled silica hydrogel slurry, 2500 g of Nalco Grade 1140 colloidal Si0₂ and 2353 g of Natka clay were Drais milled and spray dried. The spray-dried samples were then calcined for 40 minutes at 700° C.

300 g of the calcined, spray dried sample was impregnated with an aqueous solution of vanadium sulfate to give 2 wt% V. After impregnation the sample was dried at 120° C. The final material was analyzed by ICP and found to contain 2.0 wt% V, 0.39 wt% Na₂O, 4.2% SO₄. The surface area, as determined by N₂-BET, was 115 m²/g.

### Example 4

### (Preparation of 0.42 % vanadium/zeolite additive)

A vanadium,/zeolite catalyst was prepared by spray-drying a slurry of 50% USY, 30% clay and 20% silica sol. The spray-dried material was ammonium exchanged to remove the Na⁺, rare earth exchanged and then dried at 100°C. Vanadium was added by impregnation of the catalyst to incipient wetness using an aqueous vanadium oxalate solution. The amount of vanadium oxalate in solution was adjusted to a target of 0.4 wt%.

The final material was analyzed by ICP and found to contain 0.42 wt% V, 3.8 wt% RE₂O₃ and 0.27 wt% Na₂O. The surface area as determined by N₂-BET, was 375 m²/g_{.}

### Example 5

### (Catalytic Evaluation of Vanadium Supported on Al₂O₃)

The V/ Al₂O₃ additives from Example 1 were blended with a commercial FCC catalyst and steam deactivated in a fluidized bed for 4 hours at 816°C (1500° F) in 100% steam. The additive/FCC catalyst blends were designed so that the blend contained 1000 ppm V (95 wt% FCC Catalyst/5 wt% of 2%V/Al₂O₃ additive; and 98 wt% FCC Catalyst/2 wt% of 5%V/Al₂O₃ additive).

The additive/FCC catalyst blends were tested for gas oil cracking activity and selectivity using an ASTM Microactivity Test ("MAT") (ASTM procedure D-3907). The liquid product from each run was analyzed for sulfur using a gas chromatograph with an Atomic Emission Detector (GC-AED). Analysis of the liquid products with the GC-AED allows each of the sulfur species in the gasoline region to be quantified. For purposes of this example, the cut gasoline will be defined as C₅ to C₁₂ hydrocarbons that have a boiling point up to 221°C (430° F). The sulfur species included in the cut of gasoline range include thiophene, tetrahydrothiophene, C₁-C₅ alkylated. thiophenes and a variety of aliphatic sulfur species. Benzothiophene is not included in the cut gasoline range. The properties of the gas oil feed used in the MAT test are shown in the Table 1.

**Table 1**

| Properties of Vacuum Gas Oil Feed | |
|---|---|
| API Gravity | 26.6 |
| Aniline Point, °C (°F) | 83,3 (182) |
| CCR, wt% | 0.23 |
| | |
| Sulfur, wt% | 1.05 |
| Nitrogen, ppm | 600 |
| Basic Nitrogen, ppm | 310 |
| | |
| Ni, ppm | 0.32 |
| V, ppm | 0.68 |
| Fe, ppm | 9.15 |
| Cu, ppm | 0.05 |
| Na, ppm | 2.93 |

| Distillation | |
|---|---|
| IBP, °C (°F) | 181 (358) |
| 50 wt%, °C (°F) | 380 (716) |
| 99.5 wt%, °C (°F) | 610 (1130) |

The MAT data for the catalysts is shown in the Table 2; where the product selectivity was interpolated to a constant conversion of 70 wt%. The first column shows the FCC catalyst without the vanadium-based sulfur reduction additive. The next two columns show FCC catalyst blended with the 2 wt% V and 5 wt% V additives, respectively. The data shows that both vanadium additives decrease cut gasoline range sulfur 55-65% as compared to the base FCC catalyst. The coke and H₂ increase modestly for the samples that contain the vanadium additives.

**Table 2**

| MAT Product catalyst | Base FCC | 95 wt% FCC Catalyst | 98 wt% FCC |
|---|---|---|---|
| Yields | Catalyst | 5 wt% (2% V/Al₂O₃) | 2 wt% (5% V/Al₂O₃) |
| Conversion | 70 | 70 | 70 |
| Cat/Oil | 2.8 | 3.5 | 3.6 |
| | | | |
| H2 Yields, wt% | 0.06 | 0.20 | 0.22 |
| C1 + C2 Gas, wt% | 1.40 | 1.55 | 1.58 |
| | | | |
| Total C3 Gas, wt% | 4.97 | 4.97 | 5.02 |
| Propylene, wt% | 4.06 | 4.06 | 4.10 |
| Total C4 Gas, wt% | 9.96 | 10.02 | 9.94 |
| | | | |
| C5+gasoline, wt% | 51.07 | 49.83 | 50.17 |
| LCO, wt% | 25.77 | 25.85 | 25.90 |
| Bottoms, wt% | 4.13 | 4.10 | 4.20 |
| Coke, wt% | 2.55 | 3.11 | 3.18 |
| | | | |
| Cut Gasoline S, ppm | 263 | 112 | 98 |
| % Reduction in Cut | Base | 57% | 63% |
| Gasoline Sulfur | | | |

### Example 6

### (Catalytic Evaluation of V/Al₂O₃ Steamed Deactivated Together and Separately from the FCC Catalyst)

The need for transport of vanadium from the additive to the catalyst during deactivation in order to achieve good cut gasoline sulfur reduction is demonstrated in this example. The 6% V/Al₂O₃ additive from Example 2 was blended at a 4 wt% level with a FCC equilibrium catalyst (120 ppm V and 60 ppm Ni) and mildly steam deactivated for 20 hours at 732°C (1350° F) in 25% steam to simulate catalytic cracking conditions.

Separation of the additive from Ecat by skeletal density differences and analysis of the fractions by ICP shows that on the ECAT fraction, the vanadium content has increased from 120 ppm V to 2360 ppm V during the steaming process. A comparison example was made by steam deactivating the Ecat and the 6% V/ Al₂O₃ additive each separately, for 20 hours at 732°C (1350° F) in 25% steam, and then blending the additive at a 4 wt% level. The base case Ecat was also steamed for 20 hours at 1350° F in 25% steam. The steam deactivated Ecat and the Additive/FCC catalyst blends were tested for gas oil cracking and selectivity using ASTM Microactivity Test ("MAT")(ASTM procedure D-3907) as described in Example 5. The properties of the gas oil used in this example are shown in Table 1.

The MAT data for the catalyst is shown in the Table 3, where the product selectivity was interpolated to a constant conversion of 70 wt%. The first column shows data for the FCC Ecat without the vanadium based sulfur reduction additive. The second column shows data for the FCC Ecat steamed together with the V/Al₂O₃ additive. The third column shows data for the FCC Ecat and V/ Al₂O₃ additive steamed separately and then blended together. The data shows that when the additive is steamed together with the FCC catalyst (as typical of catalytic cracking process conditions) vanadium is transported from the additive to the catalyst to provide a substantial cut in gasoline sulfur reduction. The coke and H₂ increased modestly for the samples that contain the vanadium additives.

**Table 3**

| MAT Product Yield | Base Equilibrium Catalyst | 96 wt% FCC ECAT 4 wt% (6% V/Al₂O₃) Steamed Together | 96 wt% FCC ECAT 4 wt% (6% V/Al₂O₃) Steamed Separately |
|---|---|---|---|
| Conversion | 70 | 70 | 70 |
| Cat/Oil | 3.70 | 4.26 | 4.26 |
| | | | |
| H2 Yields, wt% | 0.04 | 0.09 | 0.10 |
| C1 + C2 Gas, wt% | 1.37 | 1.50 | 1.45 |
| | | | |
| Total C3 Gas, wt% | 5.07 | 5.29 | 5.15 |
| Propylene, wt% | 4.38 | 4.58 | 4.45 |
| Total C4 Gas, wt% | 10.02 | 10.44 | 10.15 |
| | | | |
| C5+gasoline, wt% | 50.94 | 49.76 | 50.10 |
| LCO, wt% | 25.38 | 25.21 | 25.16 |
| Bottoms, wt% | 4.42 | 4.57 | 4.57 |
| Coke, wt% | 2.13 | 2.48 | 2.54 |
| | | | |
| Cut Gasoline S, ppm | 525 | 359 | 521 |
| % Reduction in Cut | Base | 32 | 1 |
| Gasoline Sulfur | | | |

### Example 7

### (Catalytic Evaluation of vanadium supported on SiO2/Clay)

The 2% V/SiO₂/Clay additive from Example 3 was blended at a 5% level with a FCC Ecat (120 ppm V and 60 ppm Ni) and mildly steam deactivated for 20 hours at 732°C (1350°F) in 25% steam. As a comparison, the base Ecat was also deactivated under those conditions. The steam deactivated base Ecat and the additive FCC blends were tested for gas oil cracking activity and selectivity using an ASTM Microactivity Test (ASTM procedure D-3907) as described in Example 5. The properties of the gas oil used in this example are shown in Table 4.

The MAT data for the catalysts is shown in Table 5, where the product selectivity was interpolated to a constant conversion of 70 wt%. The data shows that the V/SiO₂/Clay additive decreases cut gasoline sulfur 42% as compared to the base case Ecat.

**Table 4**

| Properties of Vacuum Gas Oil Feed | |
|---|---|
| API Gravity | 25.3 |
| Aniline Point, °F | 178 |
| CCR, wt% | 0.21 |
| | |
| Sulfur, wt% | 1.04 |
| Nitrogen, ppm | 700 |
| Basic Nitrogen, ppm | 308 |
| | |
| Ni, ppm | 0.2 |
| V, ppm | 0.4 |
| | 3.7 |
| Fe, ppm | |
| Cu, ppm | 0 |
| Na, ppm | 0 |
| | |

| Distillation | |
|---|---|
| IBP, °C (°F) | 153,5 (309) |
| 50 wt%, °C (°F) | 397,8 (748) |
| 99.5 wt%, °C (°F) | 572,8 (1063) |

**Table 5**

| MAT Product Yields | Base Ecat | 95% Ecat 5%[2% V/SiO2/Clay] |
|---|---|---|
| Conversion | 70 | 70 |
| Cat/Oil | 3.64 | 4.05 |
| | | |
| H2 Yield | 0.05 | 0.10 |
| C1 + C2 Gas | 1.33 | 1.39 |
| Total C3 Gas, wt% | 4.53 | 4.58 |
| Total C4 Gas, wt% | 9.69 | 9.39 |
| | | |
| C5+gasoline, wt% | 51.86 | 51.56 |
| LCO, wt% | 24.61 | 23.97 |
| | | |
| Bottoms, wt% | 5.31 | 5.44 |
| Coke, wt% | 2.26 | 2.53 |
| | | |
| Cut Gasoline S, ppm | 616 | 361 |
| % Reduction in Cut Gasoline | | |
| Sulfur | Base | 42 |

### Example 8

### (Catalytic cracking performance of 6% V/Alumina versus V/zeolite catalyst)

This example shows the utility of the high vanadium-containing additive in circulating FCC riser/regenerator pilot plant testing. The high vanadium-containing additive described in Example 2 was tested in a Davison Circulating Riser pilot plant with a commercial FCC feed and equilibrium catalyst. For comparison, the vanadium/zeolite additive described in Example 4 was also tested. The equilibrium catalyst contained 332 ppm Ni and 530 ppm V. The feed properties are shown in Table 6. The DCR was operated with a riser temperature of 527°C (980°F) and a regenerator temperature of 704°C (1300°F). All the liquid products were analyzed by GC-AED for gasoline sulfur levels.

The testing results are shown in Table 7. The high vanadium-containing additive tested at a 2 wt% additive level gave 33% cut gasoline sulfur reduction as compared to the base Ecat. The vanadium/zeolite additive decreased cut gasoline sulfur 13% when used at the 22% additive level and 26% when used at the 50% additive level. The coke and hydrogen yields were marginally higher for the high vanadium-containing additive than for the base case Ecat.

**Table 6**

| Properties of Vacuum Gas Oil Feed | |
|---|---|
| API Gravity | 23.9 |
| Aniline Point, °F | 186 |
| CCR, wt% | 0.62 |
| | |
| Sulfur, wt% | 1.50 |
| Nitrogen, ppm | 1000 |
| Basic Nitrogen, ppm | 140 |
| | |
| Ni, ppm | 0.3 |
| V, ppm | 0.3 |
| Fe, ppm | 0.7 |
| Cu, ppm | 0 |
| Na, ppm | 0.9 |
| | |

| Distillation | |
|---|---|
| IBP, °C (°F) | 220,5 (429) |
| 50 wt%, °C (°F) | 417,5 (783) |
| 99.5 wt%, °C (°F) | 700 (1292) |

**Table 7**

| DCR Product Yields | Base FCC Catalyst | 78 wt% FCC Cat. 22% V/Zeolite Cat. | 50 wt% FCC Cat. 50% V/Zeolite Cat. | 98 wt% FCC Cat. 2% (6%V/Al2O3) |
|---|---|---|---|---|
| Conversion | 72 | 72 | 72 | 72 |
| Cat/Oil | 6.69 | 6.47 | 6.61 | 7.92 |
| | | | | |
| H2 Yield | 0.03 | 0.04 | 0.05 | 0.08 |
| C1 + C2 Gas | 2.41 | 2.53 | 2.63 | 2.37 |
| Total C3 Gas, wt% | 6.68 | 6.59 | 6.66 | 6.29 |
| Total C4 Gas, wt% | 12.41 | 12.06 | 12.24 | 11.79 |
| | | | | |
| C5+gasoline, wt% | 45.95 | 46.11 | 45.51 | 46.20 |
| LCO, wt% | 2059 | 20.28 | 20.15 | 20.66 |
| | | | | |
| Bottoms, wt% | 7.41 | 7.72 | 7.85 | 7.34 |
| Coke, wt% | 4.11 | 4.02 | 4.24 | 4.58 |
| | | | | |
| Cut Gasoline S, ppm | 877 | 765 | 651 | 589 |
| % Reduction in Cut | | | | |
| Gasoline Sulfur | Base case | 13 | 26 | 33 |

## Claims

1. Use of a non-molecular sieve support selected from the group consisting of refractory inorganic oxides of Groups 4, 13 and 14 of the Periodic Table and mixtures thereof, activated carbon or mixtures thereof, which support contains 1.5 to 20 weight percent of vanadium in an oxidation state greater than zero (as metal, based on total weight of the additive), as an additive in a fluid catalytic cracking process to reduce the sulfur content of liquid cracking products.

2. Use according to claim 1, wherein the support is selected from the group consisting of alumina, silica, titania, clay and mixtures thereof.

3. Use according to claim 2, wherein the support is alumina.

4. Use according to any one of the preceding claims, wherein the additive contains from 2 to 20 weight percent of vanadium (as metal, based on the weight of the additive).

5. Use according to claim 4, wherein the additive contains from 3 to 10 weight percent of vanadium (as metal, based on the weight of the additive).

6. Use according to any preceding claim, wherein the vanadium has been impregnated into or onto the surface of the support.

7. Use according to any one of claims 1 to 5, wherein vanadium has been incorporated into the support.

8. Use according to any preceding claim, wherein the additive is a separate particle additive.

9. Use according to claim 8, wherein the additive has a particle size ranging from 10 to 200 microns, preferably 20 to 120 microns and in particular 20 to 100 microns.

10. Use according to any preceding claim, wherein the additive is used in an amount sufficient to increase the amount of vanadium on the cracking catalyst by 100 to 10,000 ppm, preferably 500 to 5,000 ppm, most preferably 1,000 to 2,000 ppm, relative to the amount of vanadium initially present on the cracking catalyst.

11. Use according to any preceding claim, wherein the additive is used in an amount from 0.1 to 10 weight percent, preferably 0.5 to 5 weight percent, most preferably 2 weight percent of the cracking catalyst inventory in the fluid catalytic cracking unit.

## Patentansprüche

1. Verwendung eines Trägers, der kein Molekularsieb ist, ausgewählt aus der Gruppe bestehend aus hitzebeständigen anorganischen Oxiden der Gruppen 4, 13 und 14 des Periodischen Systems der Elemente und Mischungen derselben, Aktivkohle und Mischungen davon, wobei der Träger 1,5 bis 20 Gew.% Vanadium in einer Oxidationsstufe größer als 0 (als Metall, bezogen auf das Gesamtgewicht des Additivs) enthält, als Additiv in einem katalytischen Fließbettcrackverfahren zur Verringerung des Schwefelgehalts der flüssigen Crackprodukte.

2. Verwendung nach Anspruch 1, bei der der Träger ausgewählt ist aus der Gruppe bestehend aus Aluminiumoxid, Siliciumdioxid, Titanoxid, Ton und Mischungen davon.

3. Verwendung nach Anspruch 2, bei der der Träger Aluminiumoxid ist.

4. Verwendung nach einem der vorangehenden Ansprüche, bei der das Additiv 2 bis 20 Gew.% Vanadium (als Metall, bezogen auf das Gewicht des Additivs) enthält.

5. Verwendung nach Anspruch 4, bei der das Additiv 3 bis 10 Gew.% % Vanadium (als Metall, bezogen auf das Gewicht des Additivs) enthält.

6. Verwendung nach einem der vorangehenden Ansprüche, bei de das Vanadium in den Träger oder auf die Oberfläche des Trägers imprägniert worden ist.

7. Verwendung nach einem der Ansprüche 1 bis 5, bei der das Vanadium dem Träger einverleibt worden ist.

8. Verwendung nach einem der vorangehenden Ansprüche, bei der das Additiv ein Additiv aus separaten Teilchen ist.

9. Verwendung nach Anspruch 8, bei der das Additiv eine Teilchengröße im Bereich von 10 bis 200 µm, vorzugsweise 20 bis 120 µm und insbesondere 20 bis 100 µm aufweist.

10. Verwendung nach einem der vorangehenden Ansprüche, bei der das Additiv in einer ausreichenden Menge verwendet wird, um die Menge an Vanadium auf dem Crackkatalysator um 100 bis 10.000 ppm, vorzugsweise 500 bis 5.000 ppm und am meisten bevorzugt 1.000 bis 2.000 ppm relativ zu der Menge an Vanadium zu erhöhen, die anfänglich auf dem Crackkatalysator vorhanden war.

11. Verwendung nach einem der vorangehenden Ansprüche, bei der das Additiv in einer Menge von 0,1 bis 10 Gew.%, vorzugsweise 0,5 bis 5 Gew.% und am meisten bevorzugt 2 Gew.% des Crackkatalysatorinventars in der katalytischen Fließbettanlage verwendet wird.

## Revendications

1. Utilisation d'un support de tamisage non-moléculaire sélectionné dans le groupe consistant en oxydes inorganiques réfractaires des Groupes 4, 13 et 14 de la Table Périodique et de leurs mélanges, de charbon actif ou de ces mélanges, ledit support contenant 1,5 à 20 pour cent en poids de vanadium dans un état d'oxydation supérieur à zéro (comme métal, basé sur le poids total de l'additif), comme un additif dans un processus de craquage catalytique fluide pour réduire la teneur en soufre des produits de craquage liquides.

2. Utilisation selon la revendication 1, dans laquelle le support est sélectionné dans le groupe consistant en alumine, silice, dioxyde de titane, argile et leurs mélanges.

3. Utilisation selon la revendication 2, où le support est l'alumine.

4. Utilisation selon l'une quelconque des revendications précédentes, où l'additif contient de 2 à 20 pour cent en poids de vanadium (comme métal, basé sur le poids de l'additif).

5. Utilisation selon la revendication 4, dans laquelle l'additif contient de 3 à 10 pour cent en poids de vanadium (comme métal, basé sur le poids de l'additif).

6. Utilisation selon l'une quelconque des revendications précédentes, dans laquelle le vanadium a été imprégné dans ou sur la surface du support.

7. Utilisation selon l'une quelconque des revendications 1 à 5, où le vanadium a été incorporé dans le support.

8. Utilisation selon l'une quelconque des revendications précédentes, où l'additif est un additif particulaire séparé.

9. Utilisation selon la revendication 8, où l'additif a une taille de particule de 10 à 200 microns, de référence de 20 à 120 microns et en particulier de 20 à 100 microns.

10. Utilisation selon l'une quelconque des revendications précédentes, où l'additif est utilisé en une quantité suffisante pour augmenter la quantité de vanadium sur le catalyseur de craquage de 100 à 10 000 ppm, de préférence de 500 à 5000 ppm, selon la plus grande préférence de 1000 à 2000 ppm, relativement à la quantité de vanadium initialement présente sur le catalyseur de craquage.

11. Utilisation selon l'une quelconque des revendications précédentes, où l'additif est utilisé en une quantité de 0,1 à 10 pour cent en poids, de préférence de 0,5 à 5% en poids, selon la plus grande préférence de 2% en poids de l'inventaire de catalyseur de craquage dans l'unité de craquage catalytique fluide.
